

## UNITED STATES PATENT OFFICE.

CLARENCE J. RODMAN, OF WILKINSBURG, PENNSYLVANIA, ASSIGNOR TO WESTINGHOUSE ELECTRIC & MANUFACTURING COMPANY, A CORPORATION OF PENNSYLVANIA.

## DEOXIDIZER.

No Drawing.

Application filed December 21, 1923. Serial No. 682,075.

This invention relates to the removal of oxygen from atmospheres containing the same, and more particularly, to the removal of oxygen from closed containers, such as 5 the tanks of transformers, circuit breakers, oil switches, and the like.

In apparatus of this character, it is customary to place the transformer body, or the like, within a metal container or tank, 10 and cover the same with a high grade insulating oil. A space is left above the oil level to permit expansion thereof under normal operating conditions, and there is usually provided means whereby communication is allowed to the outside air in order 15 that upon expansion or contraction of the oil, air may be forced out or drawn in, a phenomenon which is known as breathing.

The oxygen in the air, which is breathed 20 by the transformer, gradually reacts with the oil, forming a sludge which is detrimental to the insulating properties thereof. Furthermore, it frequently occurs that there 25 is an arc formed in the apparatus which disrupts part of the oil, forming combustible gases which mix with the air above the oil and which may accidentally be united. It has occurred at various times that explosions took place with a consequent loss of the 30 apparatus and injury to the operators.

In order to prevent the detrimental effects 35 of oxygen, it has been proposed to provide an inert atmosphere in the container. One of the means was to provide a material through which all the air necessary for 40 breathing of the transformer shall pass, the material being capable of absorbing the oxygen from the air, thus rendering the atmosphere above the oil inert.

45 My invention relates to such materials, it being among the objects thereof to provide a material for deoxidizing atmospheres which shall be effective in removing the oxygen, which shall have a long life and shall not deteriorate on standing.

I have found that certain metals or mixtures of metals, and alloys in finely divided form, are capable of removing the oxygen 50 from air and are not affected by atmospheric conditions, such as humidity. Among the metals which have particularly desirable properties, are copper, lead, antimony, tellurium, cadmium, arsenic and tin.

These metals, which are lower in the electromotive series than hydrogen, do not decompose water at ordinary temperatures and only a few of these at higher temperatures. These metals tarnish or oxidize quite readily in air, and the resulting oxides are practically insoluble in water. These metals possess atomic numbers beginning with copper having an atomic number of 29 and ending essentially with tellurium having a number of 52, with the exception of one or two metals, such as bismuth and lead having atomic numbers of 82 and 81, respectively. The elements in this group have comparatively low melting points, generally below 650° C. with the exception of copper, which melts at about 1083° C.

These elements lying within the above limits, unless otherwise stated, subject themselves to a process of rapid corrosion best in the finely divided state; less than 200 mesh works most rapidly, although elements of coarser mesh operate satisfactorily, but the reactivity is correspondingly decreased. This divisibility of material does not hold for metals in the highly porous state where oxidation may be facilitated by certain salts in solution, which, when added to other constituents of the deoxygenation material give it a moist or soggy consistency. Many of these elements and oxides or other compounds thereof, are soluble in alkalis.

It has been demonstrated that these elements oxidize rapidly in the presence of monatomic anions, chlorine being suitably adapted to the process if added as a free alkali chloride, or a strongly electropositive action metal chloride, of which calcium chloride is an example. These elements subject themselves to the action of catalysts in hastening oxidation. Metalloids and carbon acting as catalysts have been found to work well, but other substances having catalytic propensities may be utilized. Organic materials such as powdered starch, flour and even activated, precipitated silica have been found to hasten the process of deoxygenation.

Although I have described my invention setting forth certain metals and alloys which are particularly desirable for the purpose, my invention is not limited to the metals named above, as other metals also have the

desired properties. For instance, some of the nobler metals may be used. Although I have mentioned the use of catalizers, it is obvious that the function of the metals will proceed to some extent without a catalizer, but I utilize the catalizers to increase the speed of the reaction and catalizers other than those mentioned may be used.

- I claim as my invention:
- 10 1. A material for deoxidizing atmospheres comprising a metal capable of oxidizing at atmospheric temperatures but incapable of decomposing water, and a substance capable of catalizing the action of said metal.
  - 15 2. A material for deoxidizing atmospheres comprising a metal capable of oxidizing at atmospheric temperatures but incapable of decomposing water, and a substance capable

of catalizing the action of said metal, both in finely divided form.

20 3. A material for deoxidizing atmospheres comprising a metal capable of oxidizing at atmospheric temperatures but incapable of decomposing water and a substance containing a monatomic anion capable of catalizing the action of said metal.

4. A material for deoxidizing atmospheres comprising a metal capable of oxidizing at atmospheric temperatures but incapable of decomposing water, and a substance containing a halogen anion capable of catalizing the action of said metal.

25 In testimony whereof, I have hereunto subscribed my name this 17th day of December 1923.

CLARENCE J. RODMAN.